

# UNITED STATES PATENT OFFICE.

PAUL RALPH HERSHMAN, OF CHICAGO, ILLINOIS, ASSIGNOR TO ARMOUR FERTILIZER WORKS, OF CHICAGO, ILLINOIS, A CORPORATION OF NEW JERSEY.

## PRODUCTION OF NITROGENOUS COMPOUNDS.

1,188,772.

Specification of Letters Patent. Patented June 27, 1916.

No Drawing. Continuation of application Serial No. 871,003, filed November 9, 1914. This application filed January 10, 1916. Serial No. 71,218.

To all whom it may concern:

Be it known that I, PAUL RALPH HERSHMAN, a citizen of Austria-Hungary, residing at Chicago, in the county of Cook and State 5 of Illinois, have invented certain new and useful Improvements in the Production of Nitrogenous Compounds, of which the following is a specification.

One of the chief objects and aims of this 10 invention is the production of nitrogenous compounds, such for example, as the nitrogenous compounds of aluminum, by an improved process or method, so as to secure by the addition of certain ingredients to the 15 mixture, an increase in the amount of nitrogen which will be combined as contrasted with the amount of nitrogen which would be taken up during the same time period without the addition of these ingredients, or, a 20 further object of the invention is to effect the combination with the nitrogen at lower temperatures in the same proportion as effected otherwise without the use of the additional ingredients or catalytic agents at 25 higher temperatures.

The advantages of this invention are secured or accomplished by adding to the mixture employed a small amount of a carrying agent capable of forming unstable compounds with nitrogen, and preferably, although not exclusively, by adding such a carrying agent as is capable of combining with nitrogen in more than one proportion. I have particularly in mind compounds of 30 that nature in which the higher proportion of nitrogen may be reduced by hydrogen to one with a lower proportion of nitrogen, possibly with an intermediate formation of ammonia.

40 The improved process or method in its preferred manner of execution is carried out as follows: A powdered mixture of aluminum oxid with at least sufficient carbon to effect its reduction, and containing from one-half (½) to five (5) per cent. by weight of a carrying-agent of the nature described, such as titanium, calcium, or those of their combinations with other elements which are susceptible to reduction by carbon, is heated to 45 a temperature of 1500 to 1600 degrees centigrade in a current of nitrogen and some hydrogen, as, for instance, generator or producer gas.

The carrying-agent employed combines

with the nitrogen and when such compound 55 is further subjected to the action of nitrogen it facilitates and aids the combination of or the reaction between the aluminum and nitrogen in the production of aluminum nitrid, or, if generator or producer gas containing 60 both nitrogen and hydrogen is used, the combination of the carrying-agent and the higher proportion of nitrogen is reduced by the hydrogen, with possibly an intermediate formation of ammonia, and, at the same 65 time, aids the combination of the nitrogen with the aluminum.

I do not wish to be strictly limited to the theory of the reaction herein advanced, as in cases of this kind, the exact reactions occurring are difficult to ascertain, but the action indicated above may be taken as a working basis. That is to say, if the current of nitrogen alone is used, the presence of the carrying-agent assists in the union of the 75 aluminum and nitrogen, while a somewhat similar result is obtained if a gas containing both nitrogen and hydrogen is employed. In both instances the use of the carrying-agent increases the amount of nitrogen taken 80 up by the aluminum and hastens the reaction.

This invention is not strictly confined to the exact ingredients specified nor to the precise proportions of parts and temperatures indicated, because these may be modified within certain limits without departure from the substance of the invention and without sacrificing any of its substantial benefits.

90 This application is a continuation of my former application, Serial No. 871,003, production of nitrogenous compounds, filed November 9, 1914.

I claim:

95 1. The method of producing nitrogenous compounds of aluminum which consists in heating in a current of nitrogen at a temperature sufficient to effect the reaction, a mixture of aluminum oxid, sufficient carbon 100 to reduce the oxid, and a carrying-agent capable of combining with nitrogen in more than one proportion, substantially as described.

105 2. The method of producing nitrogenous compounds of aluminum which consists in heating in a current of gas containing nitrogen and hydrogen at a temperature sufficient

to effect the reaction, a mixture of aluminum oxid, sufficient carbon to reduce the oxid, and a carrying-agent capable of combining with nitrogen in more than one proportion, substantially as described.

3. The method of producing nitrogenous compounds of aluminum which consists in heating in a current of gas containing nitrogen and hydrogen at a temperature sufficient

to effect the reaction, a mixture of aluminum <sup>10</sup> oxid, sufficient carbon to reduce the oxid, and a carrying-agent capable of combining with nitrogen in more than one proportion, and which in its nitrogen combination is susceptible of reduction by hydrogen, substan- <sup>15</sup> tially as described.

PAUL RALPH HERSHMAN.